

# UNITED STATES PATENT OFFICE.

MAX DICKERT, OF WERNE, GERMANY.

## METHOD OF PRODUCING WATERPROOF COATINGS ON OBJECTS WHICH ARE INFLUENCED BY HUMIDITY.

1,180,704.

Specification of Letters Patent. Patented Apr. 25, 1916.

No Drawing.

Application filed July 30, 1915. Serial No. 42,826.

*To all whom it may concern:*

Be it known that I, MAX DICKERT, a subject of the German Emperor, residing at Werne, in the Province of Westphalia, 5 Kingdom of Prussia, and German Empire, have invented certain new and useful Improvements in Methods of Producing Waterproof Coatings on Objects Which are Influenced by Humidity, of which the following 10 is a specification.

My invention relates to a method of producing a very thin coating which renders the objects provided therewith absolutely indifferent to humidity. Although this 15 method is fit for quite general purposes, the same is in particular very well adapted for coating the cartridges of sporting guns which are provided with a card-board casing.

My improved method is preferably carried out in the following manner: The object to be provided with said coating is first dipped into a solution of gutta-percha or balata, for example, in benzol, bisulfid or tetrachlorid of carbon, either colorless or 25 colored by means of a dye, said solution being preferably heated to a suitable temperature. In this way said object obtains a thin coating of said substance. Now the object is provided with a coating of cellulose acetate. To attain this end said object is dipped 30 into a suitable solution, for instance, a solution of cellulose acetate in chloroform or nitrobenzol. After vaporizing the solvent, the object is heated about half an hour to a 35 point above the degree of temperature at which the balata or gutta-percha becomes plastic, *i. e.* begins to melt.

My improved method is based upon the following considerations: Neither balata 40 nor gutta-percha is quite waterproof in small layers. This is not the case for cellulose acetate. Further, neither balata nor gutta-percha is indifferent to air. Consequently, the second coating composed of 45 cellulose acetate has a double purpose. First, said coating of cellulose acetate is intended to close the pores contained in the balata or gutta-percha layer; and secondly it has for its purpose to protect said coating 50 of balata or gutta-percha against the action of air. The combined coating becomes quite waterproof only on being heated above

the temperature at which the first layer or coating becomes plastic or semi-liquid, because, owing to the fact that the balata or 55 gutta-percha layer begins to melt, all the pores which may still exist become closed. In consequence thereof the purpose of protecting the object to be treated against the action of humidity, for example in the case 60 of cartridges provided with a card-board casing against swelling, is to a great extent attained by the co-action of both layers or coatings; however, the effect obtained is principally due to the above mentioned fact 65 that the heating takes place to such an extent that the layer of balata or gutta-percha assumes a semi-liquid condition so that the same can flow and in consequence thereof is able to fill up the pores of said 70 layer. The waterproofing which is obtainable neither with balata nor with gutta-percha alone can also not be obtained with paraffin which has been used in many cases as a protecting means against humidity. 75 Paraffin, on being used in a thin layer, does not completely protect the objects, for example cartridges, against humidity, and also paraffin has the drawback that cartridges coated therewith soils the gun-barrel after 80 repeated shooting. Lastly, I wish it to be well understood that, when in the claim I shall speak of balata alone, gutta-percha or a mixture of both is also meant as equivalent 85 for gutta-percha.

What I claim and desire to secure by Letters Patent of the United States is:—

A method of producing a waterproof coating on objects which are influenced by humidity, such as gun-cartridges provided 90 with a card-board casing, which consists in first providing the object with a layer of balata and secondly with a layer of cellulose acetate and then in heating the object above the temperature at which the first layer becomes semi-liquid or able to flow so as to 95 fill up the pores of said first-layer.

In testimony whereof I affix my signature in presence of two witnesses.

MAX DICKERT. [L.S.]

Witnesses:

HELEN NUFE,  
ALBERT NUFE.